

1,630,449

May 31, 1927.

N. B. PILLING

HEAT TREATMENT OF ELECTROLYTICALLY DEPOSITED IRON

Filed Aug. 22, 1922

Fig. 1.



Fig. 2.



Fig. 3.



WITNESSES:

C. Cochran

H. C. Biernan

INVENTOR

Norman B. Pilling

BY

Wesley L. Barr

ATTORNEY

## UNITED STATES PATENT OFFICE.

NORMAN B. PILLING, OF WILKINSBURG, PENNSYLVANIA, ASSIGNOR TO WESTINGHOUSE ELECTRIC & MANUFACTURING COMPANY, A CORPORATION OF PENNSYLVANIA.

## HEAT TREATMENT OF ELECTROLYTICALLY-DEPOSITED IRON.

Application filed August 22, 1922. Serial No. 583,468.

This invention relates to the treatment of electrolytically deposited iron, more particularly to the heat treatment thereof in order to adapt the same to a wider range of uses.

It has been proposed to reclaim undersized or worn machine parts by building up layers of electrolytically deposited iron on said parts, as such material is very adherent and may be readily applied to such elements. However, it has been found that the deposited iron is generally very brittle and may be pulverized by hammering.

It is desirable that material so deposited be modified in order to increase its workability, at the same time causing the same to become tough, and be in various stages of hardness for various applications. It is, therefore, among the objects of the present invention to so treat electrolytically deposited iron that it shall become softened and toughened and shall lose its extreme brittleness.

In practising my invention, I heat treat the deposited iron at varying temperatures, such that they induce in the iron various changes of hardness, grain structure and composition. I have found that heating or annealing the iron at a moderate temperature causes a very material increase in the hardness thereof, accompanied by a decrease in brittleness. Upon further annealing, the hardness generally decreases until, at about 900° C., the material is completely softened.

At the same time there occur changes in the crystalline structure of the iron which correspond to the changes in hardness thereof.

In the accompanying drawing constituting a part hereof.

Figure 1 is a curve showing the change in hardness with temperature;

Fig. 2 is a diagrammatic representation of the structural changes taking place during the heat treatment, and

Fig. 3 is a curve showing the evolution of hydrogen from the iron during the heat treatment.

The heating or annealing may be accomplished in any desired inert atmosphere selected to prevent excessive oxidation of the iron, since the changes brought about by heating are effected without interference by the external atmosphere. Even hydrogen may be successfully employed therefor. At

the more moderate temperatures the oxidation incurred by heating in air results in only a surface discoloration.

I have annealed various samples of electrolytically deposited iron at various temperatures, from ordinary room temperatures up to as high as 950° C. The original hardness of the deposited iron is substantially unaffected by an annealing temperature up to about 200° C. At 300° C. the hardness of the sample being annealed is increased very materially, as shown in the curve of Fig. 1, wherein an increase of over 70% in hardness is noted between 200° and 300° C. Annealing the material at successively higher temperatures results in a progressive softening from a maximum at 300° to practically complete softening at 800°. A slight increase in hardness occurs immediately after the  $A_3$  transformation at about 900° C.

During the annealing operation, the toughness of the material also undergoes a change. Annealing at various temperatures up to 300° C. results in general lessening of the brittleness of the material and a corresponding increase in the toughness thereof. At 30° the material shatters at a single hammer blow; at 200° it cracks into a number of pieces, whereas at 300° the material may be hammered and deformed in a satisfactory manner for all machine operations. Above 300° there is no apparent change in the toughness of the material.

As shown diagrammatically in Fig. 2, the electrolytically deposited iron in the annealed state is composed essentially of close, compact crystals of needle-like form. A low-temperature annealing causes a progressive change in the structure of the iron, it being manifested at about 300° C. in an indistinctness in the outlines of the crystals. Between 300° and 600° C. there is very little change in the crystal structure, but from this temperature on the crystals coalesce into large structures which are no longer needle-like. At 900° there is a complete structural change, resulting in a transformation from the large, polygonal crystals to a similar structure having small grains and very closely resembling iron which has initially been fused.

Simultaneously with the changes above noted, I have found that there occurs a de-

composition of the iron-hydrogen compound which is formed in the electrolytic deposition of the iron. The hydrogen in electrolytic iron is not merely in the free state dissolved in the iron but appears to be in the form of a well defined compound which may be decomposed by heat treatment. At a temperature as low as 90° C. the compound actively decomposes and the maximum rate of decomposition occurs between 200° and 300° C. Complete evolution of hydrogen from the iron is not accomplished before reaching the transformation point at 900° C.

My process of annealing electrolytically deposited iron results in several important changes in the material which render it more useful in various technical applications. The iron may be softened completely or may be partially hardened and simultaneously toughened. For maximum hardness and toughness, an annealing temperature of about 300° C. is utilized, whereas, for complete and rapid softening it is necessary to anneal at the relatively high temperatures of 800° to 950° C. Simultaneously with the changes in hardness and toughness there occur changes in the crystalline structure of the iron and decomposition of the hydrogen-iron compound therein.

My invention is of special utility in cases

where deposits are made upon machine parts, such as, for instance, large steel shafts and the like which become worn or are machined under size. In such instances the metal is electrolytically deposited on the shaft and the same subjected to the heat treatment at the temperature which will give the material the desired properties for the application of the shaft. By such procedure I am enabled to procure a considerable saving in such machine parts at a very low cost for repair thereof with a high degree of efficiency of the repaired part in service.

I claim as my invention:

1. A method of treating electrolytically deposited iron which consists in heating said iron to temperatures between 250° C. and about 720° C. to cause a decrease in the brittleness and an increase in the hardness thereof.

2. A method of heat treating electrolytically deposited iron which consists in heating the same to a temperature between 250° and 400° C. to cause a decrease in the brittleness and an increase in the hardness thereof.

In testimony whereof, I have hereunto subscribed my name this 17th day of August 1922.

NORMAN B. PILLING.